

# UNITED STATES PATENT OFFICE.

GEORGES ANTHEUNIS, OF GHENT, BELGIUM, ASSIGNOR TO MAX POLACHEK,  
OF CHICAGO, ILLINOIS.

## BLASTING-POWDER.

SPECIFICATION forming part of Letters Patent No. 374,921, dated December 20, 1887.

Application filed June 7, 1887. Serial No. 210,550. (No specimens.) Patented in Belgium December 31, 1884, No. 67,383, and in England January 18, 1887, No. 783.

*To all whom it may concern:*

Be it known that I, GEORGES ANTHEUNIS, a citizen of Belgium, residing at Ghent, in the Kingdom of Belgium, have invented certain new and useful Improvements in An Explosive Powder; and I do hereby declare the following to be a full, clear, and exact description of the invention, such as will enable others skilled in the art to which it appertains to make and use the same.

My invention, which was patented in Belgium on the 31st day of December, 1884, No. 67,383, and in Great Britain on the 18th day of January, 1887, No. 783, is a new safety blasting-powder, which is intended to supersede ordinary gunpowder and dynamite for all industrial purposes, being at the same time notably cheaper, quite as powerful, and perfectly harmless in handling, there being no danger 20 whatever in making and using it.

My powder is a combination of the following ingredients reduced to a fineness, sifted, and when perfectly dry triturated and mixed in revolving barrels: Mahogany sawdust, eight 25 per cent.; nitrate of potassium, fifty per cent.; nitrate of soda, sixteen per cent.; charcoal, 1.5 per cent.; sublimated sulphur, eighteen per cent.; ferro-cyanide of potassium, three per cent.; pierate of ammonium, 3.5 per cent.; 30 total, one hundred per cent.

The relative proportions of the above ingredients may of course be varied within a suitable range, according to the effect desired, and for damp climates the nitrate of soda 35 might be dispensed with altogether.

The process of manufacturing the new safety blasting-powder is as follows: The ingredients are by a separate trituration reduced to a very fine powder. Then they are, each separately,

sifted, and at last put all together in a revolving barrel and mixed until the incorporation is complete.

The powder thus manufactured is of a pale-greenish color, very fine and dry, and ready for use. It can be used in the form of compressed cartridges, as is ordinary gunpowder.

If compared to other explosives—such as gunpowder, dynamite, &c.—it offers important advantages: First, it is quite as powerful; second, it does not explode by concussion, 50 however violent, but only by ignition, and when lighted in an open space it burns briskly without exploding; third, when used for firing a mine, the stones, rocks, or minerals are smashed or divided in huge pieces, (according 55 to the quantity of powder used,) but never projected to any considerable distance; fourth, it is notably cheaper. The consequence is that my powder may be manufactured, handled, and stored without the least danger, (barring, 60 of course, the possibility of burning like any other inflammable substance, such as oil, tar, cotton, &c.,) and carried by boat or railway without any possible difficulty or objection.

Having thus described my invention, what 65 I desire to claim and secure by Letters Patent is—

The explosive compound composed of mahogany sawdust, nitrate of soda, charcoal, sublimated sulphur, ferro-cyanide of potassium, 70 and pierate of ammonium, substantially in the proportions and as specified.

In testimony whereof I affix my signature in presence of two witnesses.

GEORGES ANTHEUNIS. [L. s.]

Witnesses:

LAURENT CORNET,

LEONARD YONEKYRLS.